# EUROPEAN PATENT APPLICATION

(11) **EP 3 808 884 A1**
(43) Date of publication of application: **21.04.2021**
(21) Application number: 20818721.1
(22) Date of filing: 04.06.2020
(51) Int. Cl.: D03D 15/00, D02G 3/36, D06M 15/248, D06M 15/53, D06M 15/507, D06M 15/333, D06M 15/564, D06M 11/47, D06M 11/46

(54) **FABRIC COMPRISING COATED YARN CAPABLE OF CONTROLLING TRANSMITTANCE**

(30) Priority: 05.06.2019 KR 20190066799
(71) Applicant: Alkenz Co., Ltd., Gimhae-si, Gyeongsangnam-do 50849 (KR)
(72) Inventor: NA, Sang Hyun, Suwon-si, Gyeonggi-do 16344 (KR); JUNG, Cheol Hyun, Ulsan 44763 (KR); KANG, Hun Hee, Anseong-si, Gyeonggi-do 17572 (KR); LEE, Seop, Busan 47837 (KR); KIM, Hyo Sang, Gimhae-si, Gyeongsangnam-do 50905 (KR); CHU, Heon Seung, Jinju-si, Gyeongsangnam-do 52779 (KR)
(74) Representative: Danubia Patent & Law Office LLC
(86) International application number: PCT/KR2020/007287
(87) International publication number: WO 2020/246826

(57) **Abstract**

The present invention relates to a fabric comprising a coated yarn which is composed of a core yarn and a coating layer for coating the core yarn, and which can control transmittance, wherein the core yarn is a colored yarn having a color L value of 0-70, the coating layer is formed of a polymer resin containing an inorganic material, and the fabric has a color L value of 70 or higher, a light reflectance (R) of 40-70% and a light absorption rate (A) of 25% or higher.

## Description

### TECHNICAL FIELD

The present invention relates to a fabric comprising coated yarn capable of controlling transmittance, and more particularly, to a fabric comprising coated yarn capable of controlling transmittance, which can reduce a glare effect by controlling light transmittance through the coated yarn using a colored yarn.

### BACKGROUND ART

In general, conventional coated yarns are industrial fibers that use a coated yarn including a core yarn with a plastic material coated thereon, and are manufactured through a process of warping, weaving, and tentering. The above-described coated yarns have been used as industrial fibers such as blinds for decades.

Further, the above-described coated yarns include a core portion formed of a yarn, and a sheath portion formed by coating a polymer resin on the yarn of the core portion. Here, a polyester material having properties of excellent elasticity, less wrinkle formation, shape retention, and high strength is mainly used for the yarn forming the core portion. In particular, polyethylene terephthalate (PET) resin having physical properties of high tensile strength and low shrinkage is widely used for the yarn forming the core portion. Further, in general, the yarn forming the core portion is transparent or has a white-based color.

Plastic materials such as polyvinyl chloride (PVC), polyethylene (PE), polypropylene (PP), and thermoplastic polyurethane (TPU) are used as the polymer resin forming the sheath portion. Products that implement a color of the coated yarn by imparting a color to the polymer resin are mainly used to implement the color of the coated yarn.

In addition, a technique that imparts functionality to the fabrics made of the coated yarn by including a functional material in the polymer resin forming the sheath portion is widely used.

In this regard, Korean Patent Registration No. 0594992 discloses imparting functionality such as flame retardancy and fire retardancy to a woven fabric manufactured by coating, on an outer shell formed of a glass fiber or a polyester fiber, a coating agent including a plasticizer and a flame retardant, and a polymer material such as PVC.

Further, Korean Patent Registration No. 1286628 discloses forming a coated yarn with functionality such as flame retardancy, by including a core layer made of a polyolefin-based resin and a coating layer having a flame retardant component and the polyolefin-based resin that is the same as or different from the core layer.

The above-described coated yarn and the fabrics manufactured using the coated yarn are widely used as blind fabrics due to the properties of their materials.

Although the blind fabrics are interior products for blocking sunlight, it may be necessary for the blind fabrics to appropriately control sunlight so as to remove a glare effect due to the amount of background lighting or sunlight, thereby making the occupant's eyes comfortable within a given indoor environment.

Except for blackout blind products that are intended to block sunlight, most blind products are manufactured using bright color fabrics suitable for indoor interiors. However, these bright color products have a problem of causing a glare effect indoors due to high transmittance of sunlight or illuminating light.

In order to address the above problem, Korean Patent Application Publication No. 2018-0001531 discloses a technique of depositing any one metal selected from aluminum, copper, nickel, and silver on one or both sides of a sunscreen blind fabric. However, the metal deposition technique mentioned above has problems in that it is a process performed after manufacturing the fabrics, and thus lowers production processability and price competitiveness of the fabrics, and due to the depositing of the metal, the color or design of the fabrics cannot be freely implemented.

### DISCLOSURE OF INVENTION

### TECHNICAL PROBLEM

The present invention is to address the above-described problems in the art. The present invention is directed to providing a fabric comprising a coated yarn capable of controlling transmittance, in which a colored yarn is used as a yarn constituting the coated yarn so as to lower light transmittance such that there is no glare effect from a bright color fabric.

The present invention is further directed to providing a fabric comprising a coated yarn capable of controlling transmittance suitable for indoor blinds, in which it is possible to reduce both indoor cooling and heating energy loss due to an external environment and a glare effect due to a light source by increasing light reflectance and lowering transmittance by controlling an amount of inorganic material contained in a polymer resin for coating a core yarn of a coated yarn.

### SOLUTION TO PROBLEM

In a fabric comprising a coated yarn capable of controlling transmittance according to an embodiment of the present invention, the coated yarn is composed of a core yarn and a coating layer for coating the core yarn, wherein the core yarn is a colored yarn having a color L value of 0 to 70, the coating layer is formed of a polymer resin containing an inorganic material, and the fabric has a color L value of 70 or higher, light reflectance (R) of 40 to 70%, and light absorption rate (A) of 25% or higher, and satisfies the following equations (1) and (2):$5 \leq A / T$ $0.9 \leq R / A < 3$ wherein R refers to the light reflectance, T refers to a transmittance, and A refers to the light absorption rate.

In addition, in the fabric comprising the coated yarn capable of controlling transmittance according to an embodiment of the present invention, the fabric satisfies the following equation (3):$0.95 \leq {log}_{x} L < 5.5$ wherein x refers to an integral amount of inorganic material (phr) contained in the polymer resin, and L refers to an integer of the color L value of the core yarn.

In addition, in the fabric comprising the coated yarn capable of controlling transmittance according to an embodiment of the present invention, the core yarn is any one of multi-filament yarn, spun yarn, mono-filament yarn, or composite yarn

In addition, in the fabric comprising the coated yarn capable of controlling transmittance according to an embodiment of the present invention, the core yarn has a fineness of 50 to 1,000 denier, and the coated yarn has a fineness of 100 to 5,000 denier.

In addition, in the fabric comprising the coated yarn capable of controlling transmittance according to an embodiment of the present invention, the polymer resin forming the coating layer is any one of polyvinyl chloride (PVC) resin, polypropylene (PP) resin, polyethylene (PE) resin, polyethylene terephthalate glycol (PETG) resin, polyethylene terephthalate (PET) resin, ethylene vinyl acetate (EVA) resin, thermoplastic elastomer (TPE) resin, thermoplastic polyurethane (TPU) resin, or thermoplastic polyolefin (TPO) resin, or a mixture of two or more thereof.

In addition, in the fabric comprising the coated yarn capable of controlling transmittance according to an embodiment of the present invention, the inorganic material contained in the polymer resin is any one of antimony trioxide (Sb₂O₃), magnesium hydroxide (Mg(OH)₂), titanium dioxide (TiO₂), aluminum hydroxide (Al(OH)₃), calcium carbonate, talc, zinc oxide (ZnO), graphite, carbon black, or silica (SiO₂), or a mixture of two or more thereof.

In addition, in the fabric comprising the coated yarn capable of controlling transmittance according to an embodiment of the present invention, the inorganic material is contained in the polymer resin in an amount of 1 to 40 phr (parts per hundred resin).

### ADVANTAGEOUS EFFECTS OF INVENTION

According to the embodiments of the present invention, since the fabric comprising the coated yarn capable of controlling transmittance can increase the light absorption rate and lower the transmittance by using the colored yarn as the core yarn and including inorganic materials in the coating layer, the glare effect from bright color fabrics can be removed.

In addition, according to the embodiments of the present invention, since the fabric comprising the coated yarn capable of controlling transmittance can reduce both indoor cooling and heating energy loss due to an external environment and the glare effect from a light source by increasing the light reflectance and lowering the transmittance, the fabric can be suitable for indoor blinds.

### BEST MODE FOR CARRYING OUT THE INVENTION

Hereinafter, the preferred embodiments of the present invention will be described in detail. In describing the present invention, detailed descriptions of related known functions or configurations are omitted so as not to obscure the subject matter of the present invention.

Throughout this specification, terms of approximation such as "about", "substantially", and the like, are used to mean "at, or close to" given numerical values when manufacturing and material tolerances inherent in the stated meanings are given, and are used to prevent unscrupulous infringers from unfairly using the content referring to the exact or absolute numerical values mentioned to aid in the understanding of the present invention.

The present invention relates to a fabric comprising a coated yarn which is composed of a core yarn and a coating layer for coating the core yarn,

The core yarn constituting the coated yarn according to an embodiment of the present invention is formed of a colored yarn having a color L value of 0 to 70, and the coating layer is formed of a polymer resin containing an inorganic material.

Since the core yarn has the color L value of 0 to 70 and thus absorbs light, it may act to lower transmittance of the fabric manufactured with the coated yarn.

The core yarn accommodates any color having the color L value of 0 to 70, and may use any one of multi-filament yarn, spun yarn, mono-filament yarn, or composite yarn.

The core yarn does not have a limited fineness. However, when used for blinds, considering the weight of the fabric, it is preferable to use the core yarn having a fineness of 50 to 1,000 denier, and it is preferable for the coated yarn to have a fineness of 100 to 5,000 denier.

Any resin capable of coating the core yarn may be used as a polymer resin forming the coating layer for coating the core yarn, and for example, any one of polyvinyl chloride (PVC) resin, polypropylene (PP) resin, polyethylene (PE) resin, polyethylene terephthalate glycol (PETG) resin, polyethylene terephthalate (PET) resin, ethylene vinyl acetate (EVA) resin, thermoplastic elastomer (TPE) resin, thermoplastic polyurethane (TPU) resin, or thermoplastic polyolefin (TPO) resin, or a mixture of two or more thereof may be used as the polymer resin.

In order to supplement the properties and enhance the functionality of the polymer resin, it is preferable to use a mixture of two or more different types of polymer resins.

In addition, the polymer resin may additionally contain a plasticizer, a lubricant, and the like to enhance processability, and may additionally contain functional materials such as flame retardants, antibacterial agents, and UV stabilizers to enhance the functionality of the coated yarn.

Any inorganic material capable of reflecting or absorbing light may be used as the inorganic material contained in the polymer resin, and for example, any one of antimony trioxide (Sb₂O₃), magnesium hydroxide (Mg(OH)₂), titanium dioxide (TiO₂), aluminum hydroxide (Al(OH)₃), calcium carbonate, talc, zinc oxide (ZnO), graphite, carbon black, or silica (SiO₂), or a mixture of two or more thereof, may be used as the polymer resin.

As the amount of the inorganic material contained in the polymer resin increases, light reflectance also increases, thereby improving the color L value of the fabric. However, when too much inorganic material is contained in the polymer resin, texture and price competitiveness of the fabric may be lowered. Accordingly, it is preferable that the inorganic material is contained in the polymer resin in an amount of 1 to 40 phr (parts per hundred resin).

It is possible to increase the amount of the inorganic material contained in the polymer resin to improve the color L value of the fabric, but if the amount of the inorganic material exceeds 40 phr, the physical properties of the coated yarn may deteriorate. Accordingly, it is preferable that the inorganic material is contained in the polymer resin in an amount of 40 phr or less.

The fabric comprising the coated yarn composed of the core yarn which is a colored yarn having the color L value of 0 to 79 and the coating layer which is the polymer resin containing the inorganic material, as described above, has a color determined according to a pigment of the coating layer.

It is preferable that even if the fabric has a color with the color L value of 70 or higher, it has a reduced light transmittance due to a light reflectance (R) of 40 to 70% and a high light absorption rate (A) of 25% or higher, and satisfies the following equations (1) and (2):$5 \leq A / T$ $0.9 \leq R / A < 3$ wherein R refers to the light reflectance, T refers to the transmittance, and A refers to the light absorption rate.

Equation (1) indicates that the transmittance (T) of the fabric according to the embodiment of the present invention is 5 times or more lower than the light absorption rate (A) thereof. Accordingly, when the light reflectance (R) is constant, it is possible to control the glare effect from the fabric due to the light source by controlling the light absorption rate (A) in inverse proportion to the transmittance (T).

Equation (2) indicates the relationship between the light reflectance and the light absorption rate, and the light reflectance of the fabric is a value representing sharpness or beauty of the fabric appearance.

Since when the light reflectance is too low, sharpness or beauty of the fabric appearance may be lowered, but when the light reflectance is too high, the glare effect from the fabric due to the light source may increase, it is preferable to keep the light reflectance within a certain range. That is, when the light reflectance (R) and the light absorption rate (A) satisfy 0.9<R/A<3, it is possible to prevent the glare effect without causing deterioration of the fabric appearance.

The light reflectance, the transmittance, and the light absorption rate of the fabric according to the embodiment of the present invention are physical property values that may be controlled according to the color L value of the core yarn and the amount of inorganic material (phr) contained in the polymer resin.

Although it is possible to increase the light absorption rate and lower the transmittance of the fabric through the color L value of the core yarn, the color L value of the fabric may be lowered. In addition, although it is possible to lower the transmittance by increasing the light reflectance and the light absorption rate by increasing the amount of the inorganic material contained in the polymer resin, the texture and price competitiveness of the fabric may be lowered due to the increased amount of inorganic material contained the polymer resin. Accordingly, since it is possible to control the color L value, the light reflectance, and the transmittance of the manufactured fabric by controlling the color L value of the core yarn and the amount of inorganic material contained in the polymer resin, it is preferable that the following equation (3) is satisfied in the present invention:$0.95 \leq {log}_{x} L < 5.5$ wherein x refers to an integral amount of inorganic material (phr) contained in the polymer resin, and L refers to an integer of the color L value of the core yarn.

Equation (3) is a log value based on the color L value of the core yarn and the amount of inorganic material contained in the polymer resin. Here, when the log value is less than 0.95, this indicates that an excess of the inorganic material is contained in the polymer resin in consideration of the light reflectance and the transmittance. However, when the log value is greater than 5.5, since too little inorganic material is contained in the polymer resin to control the transmittance, the glare effect may occur.

According to the embodiment of the present invention, by controlling the color L value of the core yarn and the amount of inorganic material contained in the polymer resin within the range of Equation (3), occurrence of the glare effect from the bright color fabrics can be lowered and thus the user's comfort can be improved.

In addition, according to the embodiment of the present invention, by controlling the light reflectance and the transmittance, the glare effect caused by the light source can be lowered, and thus the bright color fabrics can be suitable for indoor blinds.

Hereinafter, a method for manufacturing the fabric comprising the coated yarn capable of controlling transmittance according to an embodiment of the present invention is described, but it should not be understood that the present invention is limited to the embodiment.

⊚ Measurement of the transmittance based on the inorganic material

50 parts by weight of polyvinyl chloride (PVC) resin, 20 parts by weight of ethylene vinyl acetate (EVA) resin, 27 parts by weight of plasticizer (DOTP), 0.5 parts by weight of lubricant (zinc stearic acid), 0.5 parts by weight of antibacterial agent (BAC-300Z), and 2 parts by weight of an ultraviolet stabilizer (benzophenone-based) were mixed to provide a mixture of resins for forming the coating layer, and then 0 to 20 phr of zinc oxide (ZnO) and titanium dioxide (TiO₂) were included in the mixture of resins to manufacture a film with a thickness of 1 mm. The measurement of the transmittance of the film is shown in Table 1 below.

**[Table 1]**

| Amount of inorganic material (phr) | Transmittance of zinc oxide (%) | Transmittance of titanium dioxide (%) |
|---|---|---|
| 0 | 15 | 15 |
| 1 | 7 | 6 |
| 2 | 5 | 5 |
| 3 | 3.5 | 3 |
| 5 | 1.7 | 1.5 |
| 10 | 0.6 | 0.5 |
| 15 | 0.1 | 0.1 |
| 20 | 0.1 | 0.1 |

As can be seen in Table 1, since the transmittance of both zinc oxide (ZnO) and titanium dioxide (TiO₂) is lowered as the amount of inorganic material contained in the polymer resin increases, it is possible to control the transmittance of the film by controlling the amount of inorganic material.

⊚ Manufacture of the fabric comprising the coated yarn capable of controlling transmittance

### Embodiments 1 to 17

250D/48F, polyester dope dyed yarn was used as the core yarn. Further, 50 parts by weight of polyvinyl chloride (PVC) resin, 20 parts by weight of ethylene vinyl acetate (EVA) resin, 27 parts by weight of plasticizer (DOTP), 0.5 parts by weight of lubricant (zinc stearic acid), 0.5 parts by weight of antibacterial agent (BAC-300Z), and 2 parts by weight of an ultraviolet stabilizer (benzophenone-based) were mixed to provide a mixture of resins, and the mixture of resins was used as the polymer resin of the coating layer. Further, titanium dioxide was included as the inorganic material in the mixture of resins.

Coated yarn of about 1,000D was manufactured by coating the mixture of resins on the core yarn at a coating speed of 500 to 1000 m/min at 150 to 180 °C using a single extrusion coating machine. During the coating process, in a state where the yarn was fixed to a winder after being passed through a nozzle, the yarn was yarn-coated by injecting the coating material composition into a hopper of an extruder and melt-extruding the yarn through the extruder.

The fabric comprising the coated yarn capable of controlling transmittance according to the embodiment of the present invention was manufactured using the coated yarn manufactured through the above-described process.

Table 2 shows control of the color L value of the core yarn and the amount of inorganic material contained in the polymer resin according to Embodiments 1 to 17.

### Comparative Examples 1 to 4

As shown in Table 2, the fabrics according to Comparative Examples 1 to 4 were manufactured in the same manner as in Embodiment 1, except that the core yarn having a color L value of 90 was used and the amount of inorganic material contained in the polymer resin was controlled.

Optical properties in Embodiments and Comparative Examples

Measurement of the color L value, the light reflectance, the transmittance, the light absorption rate, and the glare class of the fabric manufactured according to Embodiments 1 to 17 and the Comparative Examples 1 to 4 are shown in Table 2, respectively.

The color L value of the core yarn, and the color L value, the light reflectance, the transmittance and the light absorption rate of the fabric were measured using a Konica Minolta CM-5 spectrophotometer and a PerkinElmer Lambda UV/VIS/NIR spectrophotometer, and the glare class of the fabric was measured using a test method according to European EN 14501. The log value was calculated according to the following equation:$Log value = {log}_{x} L$ wherein x refers to an integral amount of inorganic material (phr) contained in the polymer resin, and L refers to an integer of the color L value of the core yarn.

**[Table 2]**

| Embodiment | Core yarn L value | Amount of inorganic material (phr) | Fabric L value | Light reflectance (%) | Transmittance (%) | Light absorption rate (%) | Glare class | Log value |
|---|---|---|---|---|---|---|---|---|
| Embodiment 1 | 18 | 2 | 77 | 38 | 3 | 59 | 3 | 4.17 |
| Embodiment 2 | 18 | 5 | 82 | 53 | 4 | 43 | 3 | 1.8 |
| Embodiment 3 | 18 | 10 | 84 | 58 | 5 | 37 | 3 | 1.26 |
| Embodiment 4 | 18 | 15 | 89 | 62 | 3 | 36 | 3 | 1.07 |
| Embodiment 5 | 18 | 20 | 90 | 64 | 3 | 33 | 3 | 0.96 |
| Embodiment 6 | 18 | 25 | 91 | 63 | 3 | 34 | 3 | 0.90 |
| Embodiment 7 | 32 | 2 | 76 | 40 | 4 | 56 | 3 | 5 |
| Embodiment 8 | 32 | 5 | 83 | 54 | 6 | 40 | 3 | 2.15 |
| Embodiment 9 | 32 | 10 | 90 | 55 | 4 | 41 | 3 | 1.51 |
| Embodiment 10 | 32 | 15 | 91 | 62 | 4 | 35 | 3 | 1.28 |
| Embodiment 11 | 32 | 25 | 93 | 65 | 3 | 32 | 3 | 1.08 |
| Embodiment 12 | 32 | 35 | 93 | 67 | 3 | 31 | 3 | 0.97 |
| Embodiment 13 | 32 | 45 | 93 | 67 | 3 | 31 | 3 | 0.91 |
| Embodiment 14 | 68 | 2 | 83 | 45 | 8 | 47 | 2 | 6.09 |
| Embodiment 15 | 68 | 5 | 85 | 55 | 5 | 40 | 3 | 2.62 |
| Embodiment 16 | 68 | 10 | 89 | 57 | 5 | 38 | 2 | 1.83 |
| Embodiment 17 | 68 | 15 | 90 | 62 | 4 | 35 | 3 | 1.56 |
| Comparative Example 1 | 90 | 2 | 92 | 63 | 26 | 11 | 1 | 6.49 |
| Comparative Example 2 | 90 | 5 | 93 | 54 | 18 | 28 | 1 | 2.8 |
| Comparative Example 3 | 90 | 10 | 93 | 65 | 15 | 20 | 1 | 1.95 |
| Comparative Example 4 | 90 | 15 | 93 | 65 | 10 | 25 | 1 | 1.66 |

As can be seen in Table 2, when the color L value of the core yarn is 68 or less, a light reflectance (R) of 40 to 70%, a light absorption rate (A) of 25% or higher, and a 3-class glare can be achieved by controlling the amount of inorganic material contained in the polymer resin. That is, as can be seen in Embodiments 1 to 5, 6 to 13, and 14 to 17, respectively, when the color L value of the core yarn is the same, as the amount of inorganic material contained in the polymer resin increases, the color L value and the light reflectance of the fabric also increase.

In addition, as can be seen in Comparative examples 1 to 4, when the color L value of the core yarn is 90, even if the amount of inorganic material contained in the polymer resin is increased, it is preferable that the transmittance is 10% or higher, the glare class is 1, and the color L value of the core yarn is 70 or less.

Embodiment 6, which has a log value of less than 0.95, does not have a significant difference in the color L value of the fabric, the light reflectance, the transmittance, and the glare class compared to Embodiments 4 and 5, which used the same core yarn. Therefore, it can be seen that in Embodiment 6, an excessive amount of inorganic material was contained in the polymer resin in consideration of the color L value of the fabric, the light reflectance, the transmittance, and the glare class.

Likewise, it can be seen that in Embodiment 13, which has a log value of less than 0.95, an excessive amount of inorganic material was contained in the polymer resin in consideration of the color L value of the fabric, the light reflectance, the transmittance, and the glare class, when compared to Embodiments 10 and 11.

Further, in Embodiment 14, which has a log value of more than 5.5, the amount of inorganic material contained in the polymer resin is low compared to the color L value of the core yarn, so the transmittance is high and the glare class is 2, and thus the glare effect occurs.

Accordingly, it can be seen that when the log value is in the range of 0.95 to 5.5, the amount of inorganic material contained in the polymer resin is controlled while maintaining a satisfactory light reflectance, transmittance, and glare class.

## Claims

1. A fabric comprising a coated yarn capable of controlling transmittance, the coated yarn being composed of a core yarn and a coating layer for coating the core yarn, **characterized in that**:
the core yarn is a colored yarn having a color L value of 0 to 70, and the coating layer is formed of a polymer resin containing an inorganic material, and
the fabric has a color L value of 70 or higher, a light reflectance (R) of 40 to 70%, and a light absorption rate (A) of 25% or higher, and satisfies the following equations (1) and (2): $5 \leq A / T$ $0.9 \leq R / A < 3$ wherein R refers to the light reflectance, T refers to a transmittance, and A refers to the light absorption rate.

2. The fabric according to claim 1, **characterized in that** the fabric comprising the coated yarn satisfies the following equation (3): $0.95 \leq {log}_{x} L < 5.5$ wherein x refers to an integral amount of inorganic material (phr) contained in the polymer resin, and L refers to an integer of the color L value of the core yarn.

3. The fabric according to claim 1, **characterized in that** the core yarn is any one of multi-filament yarn, spun yarn, mono-filament yarn, or composite yarn.

4. The fabric according to claim 1, **characterized in that** the core yarn has a fineness of 50 to 1,000 denier, and the coated yarn has a fineness of 100 to 5,000 denier.

5. The fabric according to claim 1, **characterized in that** the polymer resin forming the coating layer is any one of polyvinyl chloride (PVC) resin, polypropylene (PP) resin, polyethylene (PE) resin, polyethylene terephthalate glycol (PETG) resin, polyethylene terephthalate (PET) resin, ethylene vinyl acetate (EVA) resin, thermoplastic elastomer (TPE) resin, thermoplastic polyurethane (TPU) resin, or thermoplastic polyolefin (TPO) resin, or a mixture of two or more thereof.

6. The fabric according to claim 1, **characterized in that** the inorganic material contained in the polymer resin is any one of antimony trioxide (Sb₂O₃), magnesium hydroxide (Mg(OH)₂), titanium dioxide (TiO₂), aluminum hydroxide (Al(OH)₃), calcium carbonate, talc, zinc oxide (ZnO), graphite, carbon black, or silica (SiO₂), or a mixture of two or more thereof.

7. The fabric according to claim 1, **characterized in that** the inorganic material is contained in the polymer resin in an amount of 1 to 40 phr (parts per hundred resin).
